

# UNITED STATES PATENT OFFICE.

CORNELIUS CRONIN, OF KINGSTON, AND GWILYM EDWARDS, OF EDWARDSVILLE, PENNSYLVANIA.

## FUEL.

SPECIFICATION forming part of Letters Patent No. 498,629, dated May 30, 1893.

Application filed December 9, 1892. Serial No. 454,562. (No specimens.)

*To all whom it may concern:*

Be it known that we, CORNELIUS CRONIN, of Kingston, and GWILYM EDWARDS, of Edwardsville, in the county of Luzerne and State 5 of Pennsylvania, have invented a new and useful Improvement in Fuel, of which the following is a specification.

Our invention is in the nature of a new artificial fuel to be composed of several ingredients, and molded or compressed into bricks, blocks, or lumps, for use in stoves, furnaces, &c.

To make one ton of two thousand pounds we take of culm, seventeen hundred and 15 ninety-two pounds; wood pulp, one hundred and fifty pounds; ground limestone, fifty pounds; crude petroleum, eight pounds. These ingredients may be used in a slightly varying proportion, a little more or a little 20 less of each ingredient making no substantial difference in the product. We therefore do not confine ourselves to the exact proportions given. The culm, or comminuted coal, is the chief combustible ingredient. The 25 wood pulp is used as a fibrous binder to hold

the culm together in a mass, being itself also combustible. The ground limestone by its refractory mineral nature gives a brilliancy to the fire, and the petroleum is used for promoting combustion and facilitating the ignition of the mass. These ingredients are ground together and molded or compressed into blocks, lumps, or bricks.

To facilitate the adhesion and mixing of the mass a variable proportion of water may be 35 added depending upon the dampness of the culm.

Having thus described our invention, what we claim as new, and desire to secure by Letters Patent, is—

A composition of matter for the production 40 of artificial fuel consisting of culm, wood pulp, ground limestone, and crude petroleum, mixed in or about the proportions described.

CORNELIUS CRONIN.  
GWILYM EDWARDS.

Witnesses:

C. W. BOONE,  
W. M. VAN HORN.